

# UNITED STATES PATENT OFFICE.

KOTARO KONAGAI, OF TOKYO, JAPAN.

## WATERPROOF PAPER.

1,307,405.

Specification of Letters Patent. Patented June 24, 1919.

No Drawing.

Application filed November 8, 1918. Serial No. 261,689.

To all whom it may concern:

Be it known that I, KOTARO KONAGAI, a subject of the Emperor of Japan, and a resident of No. 27 1-chome, Motozono-Cho, Kojimachi-Ku, city of Tokyo, Empire of Japan, merchant, have invented a new and useful Improvement in Waterproof Paper, of which the following is a specification.

This invention relates to certain improvements in the manufacture of impermeable papers for use in making buckets, molds, and other containers, and consists in first immersing in a bath of gelatin solution the paper to be treated, making the solution insoluble by applying thereon a mixed solution of chrome alum solution and ammoniacal alum solution, and subsequently coating the paper with a second mixture consisting of castor oil, tung oil and lead or zinc salt, 20 as hereinafter described and claimed. The invention has for its object to obtain an impermeable paper which is smooth and without wrinkles and which has the resistance required for the purpose for which it is to 25 be used, and which is water-proof in character.

In carrying out my invention, a sheet of paper is first coated with vegetable paste, preferably bracken paste, and is then immersed in a bath of gelatin solution. This bracken paste is made of the root of the edible fern, known as bracken, especially the *Pteris Ciquitina*. This root is firstly dried, ground to powder, mixed with water, and 30 finally filtered through cotton to precipitate a sticky mass of paste. When the sheet is completely impregnated, I proceed to coat it with a mixture of chrome alum solution and ammoniacal solution, in order to make 35 the gelatin solution previously applied insoluble. This forms on the face of the paper a bed or base. I also prepare a paint by mixing 5 grams of castor oil with 5 grams of lead oxid, boiling to suitable extent, adding thereto 40 grams tung oil, heating the 40 mixture for about one hour to a temperature between 180 and 200 degrees Fahrenheit, further adding thereto 5 grams of iron oxid, and finally heating it to a temperature between 45 180 and 200 degrees Fahrenheit for

about one half of an hour. The mixture thus prepared, which may be diluted with pine oil, is then applied in an appropriate manner over the base hereinbefore described.

In order to insure success in the treatment of the paper and to attain the most efficient result, I cause the said mixture already applied upon the base to be covered with an additional layer of a compound which I prepare by mixing 5 grams of castor oil with 5 grams of white lead, heating it for about one half of an hour to a temperature preferably slightly lower than 200 degrees Fahrenheit, adding thereto 10 grams of zinc 60 oxid, 20 grams of tung oil, 15 grams of boiled linseed oil, subsequently heating to a temperature between 180 and 200 degrees Fahrenheit for about 2 hours, which, when diluted with pine oil is painted in an appropriate manner over the first coat.

In addition to the above ingredients of my second mixture compound, I sometimes mix with them a suitable quantity of zinc oxid and infusorial earth, and finish with a 75 final coating of caoutchouc solution.

The use of the ordinary tung oil alone often makes the face of the paper wrinkled, due to its speedy drying nature, which defect I am enabled to overcome by moderating to the required extent the drying property of the oil before the proper driers are added.

What I claim is:—

The process of making paper impermeable to water, and which consists in first covering the paper with gelatin solution, rendering the gelatin insoluble, then coating with a mixture of castor oil, lead oxid, tung oil and iron oxid, and subsequently coating over the 80 said mixture with a second mixture consisting of castor oil, white lead, zinc oxid, tung oil and linseed oil.

In testimony whereof I affix my signature in the presence of two witnesses.

KOTARO KONAGAI. [L.S.]

Witnesses:

J. McD. GARDINER,  
H. YASUMURA.